# EUROPEAN PATENT APPLICATION

(11) **EP 0 255 051 A1**
(43) Date of publication of application: **03.02.1988**
(21) Application number: 87110693.6
(22) Date of filing: 23.07.1987
(51) Int. Cl.: H01F 1/33

(54) **Flame retardant bond magnet**

(30) Priority: 25.07.1986 JP 176330/86
(71) Applicant: KANEGAFUCHI KAGAKU KOGYO KABUSHIKI KAISHA, Kita-ku Osaka-shi Osaka-fu 530 (JP)
(72) Inventor: Sakauchi, Takashi Kanegafuchi kagaku Kogyo K.K., Ohtsu-shi Shiga-ken (JP); Tomoda, Naohisa Kanegafuchi kagaku Kogyo K.K., Ohtsu-shi Shiga-ken (JP); Satoh, Kenji Sumitomo Metal Mining Co., Ltd., Tokyo-to (JP)
(74) Representative: Grünecker, Kinkeldey, Stockmair & Schwanhäusser Anwaltssozietät

(57) **Abstract**

The present invention provides a flame retardant bond magnet composed of a flame retarder and an organic binder in addition to alloy magnet powders with mean grain size 10µm or less represented by a general formula RM₅ (where R denotes a rare earth metal element, and M a transition metal element), which is coated on their surfaces with an oxidation resistant inorganic substance. The flame retardant bond magnet of this invention is finding wide uses in electric equipment as sensor field magnets, various drive magnets, convergence correction magnets, etc.

## Description

### BACKGROUND OF THE INVENTION

### 1. Field of the invention

The present invention relates to a flame retardant bond magnet formed of rare earth-cobalt base alloy magnet powders and more particularly provides a highly flame retardant bond magnet which will find wide uses in electric equipment as sensor field magnet, various drive magnet, convergence correction magnet, etc., and which is produced by coating said alloy magnet powders with an oxidation resistant inorganic substance.

### 2. Description of the prior art

Alloy magnets of rare earth metals and transition metals as their main components (hereinafter referred to as rare earth magnets) are finding uses as high performance magnets, because of their high energy products and small magnetic flux density temperature coefficients, but they have a drawback on account of low mechanical strength and to remedy this situation, bond magnets have been put on the market. These rare earth magnet powders are susceptible to oxidation. Thus well-known rare earth bond magnets are liable to combustion. Particularly when rare earth magnet powders represented by a general formula RM₅ (where R stands for a rare earth metal element, and M a transition metal element) are used, they need to be prepared as fine grains with mean grain size roughly 10µm or less for development of high magnetic characteristic, on account of the coercive force producing mechanism of said magnetic powders. Accordingly, the surface area of said magnet powders is very large and, therefore, the oxidation resistance or the combustion resistance of the bond magnet is very small. Recently, there has bee proposed a method of improving the combustion resistance by coating said magnet powder surfaces with some organic compound which has affinity to silane coupling agent or dyes or other inorganics, but such a method is quite inadequate where improvement in the combustion resistance is concerned. Thus it is the present situation that effective measures for improvement in rare earth bond magnets having adequate flame retardancy have yet to be proposed.

### SUMMARY OF THE INVENTION

The object of this invention is to provide a bond magnet excellent in flame retardancy.

Other objects and advantages of this invention will become apparent from the following detailed description:

The present inventors, as a result of repetitive assiduous studies with a view to attainment of the aforementioned object, have realized a bond magnet excellent in combustion resistance (flame retardancy) even by using rare earth magnet powders with mean grain size less than 10µm, which has led to this invention.

### DETAILED DESCRIPTION OF THE INVENTION

The present invention covers flame retardant bond magnet comprising alloy magnet powders with mean grain size not greater than 10µm represented by a general formula RM₅ (where R designates a rare earth metal element, and M a transition metal element), which is coated on their surfaces with an oxidation resistant inorganic substance, a flame retarder and an organic binder.

The rare earth magnet powders used according to this invention are represented by a general formula RM₅. Where R denotes samarium, praceodymium, cerium, neodymium, yttrium and other rare earth metal elements, including mixtures of samarium with other rare earth metal elements and misch metal, etc.; M designates cobalt and other transition metal elements; as these elements, mixtures of cobalt/iron or these with copper, zirconium, etc., added may be preferably utilized. Particularly useful in industrial applications are samarium - cobalt alloy magnet powders. Said rare earth magnet powders normally need to be reduced in their mean grain size to 10 µm or less in order to achieve magnetic characteristic. For this reason, the area of the active surfaces of said powders originally susceptible to oxidation notably increases and, as a consequence, they are highly inflammable at the flame temperature. Therefore, bond magnets produced from such rare earth magnet powders are liable to combustion and adequate flame retardancy can not be imparted even by adding large amounts of flame retarders. Accordingly, in order to acquire a rare earth bond magnet excellent in flame retardancy, it is necessary to make the rare earth magnet powders themselves oxidation resistant. Various methods may be contemplated to attain this.

A first of such methods is a method comprising coating the powder surfaces with organic compounds having affinity with said magnet powder surfaces. This method is scarcely effective for imparting flame retardancy, as above described. A second method comprises exposing alloy magnet powders to air under a high temperature condition, thereby forming an oxide layer on the powder surfaces. By this method, the magnetic characteristic of the bond magnet thus obtained is impaired and, moreover, dispersion in the oxide layer thickness is large. Thus this method can hardly be said advantageous.

A third method involves this invention. This method comprises coating the surfaces of said alloy magnet powders with a fine grained inorganic substance which has high oxidation resistance. By this method, sufficient anti-oxidation stability to make flame retardant the finally obtained bond magnet can be realized without impairing the magnetic characteristic inherent to the rare earth magnet powders. In the following description, the aforementioned rare earth magnet powders having no coating layer are called "magnet powders", and those having such coating layers "treated magnet powders".

Various materials may be utilized as the coating layer to be formed on magnet powders. Such materials may include, for example, chrome, nickel, copper, zinc, silver, tin, gold and other metals; nickel - chrome alloy, nickel - copper alloy and other alloys, silicates, borates, phosphates, borophosphates and other inorganics represented by inorganic glass. More particularly, lithium, sodium, potassium and ammonium silicates may be illustrated as silicates.

For coating magnet powders with the aforementioned metals or alloys, such metal film forming techniques as electroless plating, vapor deposition, spattering, etc., may be utilized. Representative of such methods is the electroless plating. Magnetic powders are dispersed in an electroless plating solution which is commercially available, which violently stirring them; the stirring is continued until the color peculiar to the metal ion in the plating solution disappears; thereafter, the powders are filtered and cleaned, yielding the intended treated magnet powders. The most representative is nickel plating. Such a metal coating layer's structure is particularly fine grained and even a relatively small amount of coating has a satisfactory specified effect, but on industrial scale, the treating facility price and the required treating time is relatively large, with a result that the manufacturing cost tends to be high. On the other hand, for coating inorganic salt, such a simple and easy method as forming a fine grained coating of said inorganic salt on the magnet powder surfaces by adding a hardener, while dispersing magnet powders in an aqueous medium in which the inorganic salt is dissolved beforehand. This method is quite preferable in industrial applications, involving only a simple process and requiring short treating time. As the hardeners, silicofluorides; mineral acids; oxides or salts of zinc, magnesium, zirconium, potassium, aluminum and other polyvalent metals and organic solvents, etc., may be illustrated. In the final analysis, the intended flame retardancy of the bond magnets will vary depending on the content and grain size of magnet powders, material of the magnet powder coating layer, type of binder, type and amount of flame retarder used. Accordingly, the amount of the coating layer in the treated magnet powders required can not be unconditionally defined, varying depending on the flame retardancy level of the bond magnet, type of the coating layer, binder and flame retarder, and the content and grain size of the magnet powders, but generally, at least 0.5% by volume of this layer in the treated magnet powders is necessary. If it is less than 0.5% by volume, the thickness of the coatig layer is too small, or the coating is imperfect, or further, sometimes only inadequate flame retardancy is achieved, depending on the material of the organic binder or the treated magnet powder content in the bond magnet. On the other hand, if the volume proportion of the coating layer in the treated magnet powders are too large, the amount of the treated magnet powders required for realizing the proper amount of magnet powders determined by the magnetic characteristic required for the bond magnet will increase, resulting in impairment of the moldability and mechanical strength of the bond magnet. Besides, forming the coating layer beyond the required amount will bring about no further increase in the effect of flame retardancy improvement and so is not advantageous. Accordingly, the volume proportion of the coating layer should desirably be limited to the minimum where the desired flame retardancy should be 1 - 40% by volume of the treated magnet powders, more preferably, 2 - 15% by volume.

The organic binder used according to this invention shall be arbitrarily selected from universally used thermoplastic resins or thermosetting resins or rubber. However, resins mainly composed of polyolefin or polyalkyl methacrylate or dienic synthetic rubbers which require very large amounts of flame retarders for attaining high flame retardancy are not recommendable. As organic binders used according to this invention, polyvinyl chloride, vinyl chloride/vinyl acetate copolymer, polystyrene, acrylonitrile/styrene copolymer, 6-polyamide, 11-polyamide, 12-polyamide, polyethylene terephthalate, polybutylene terephthalate, polyphenylene oxide, polystyrene denatured polyphenylene oxide, polycarbonate, polysufone, polyphenylene sulfide, polyallylate, thermoplastic polyimide, chlorinated polyethylene, chloroprene rubbers, phenol resins, unsaturated polyester resins and epoxy resins, etc., may be illustrated.

The amount of treated magnetic powders used in the bond magnet of this invention may be varied over a wide ranges depending on the objects. A commercially effectively utilizable range of the powders should ultimately be 15 - 85% by volume of the formulation used for molding the magnet, the balance to be composed of the organic binder and the flame retarder. If their amount exceeds 85% by volume, the product can not be put to practical use because of very small mechanical strength, even when molded by any commercially applicable method, while under 15% by volume, practically useful magnetic characteristic can not be achieved. When the amount of the treated magnetic powders used exceeds about 70% by volume, the compression molding method should be used. When it is below 70% by volume, almost all molding methods including injection, extrusion and compression molding, etc., may be utilized. The smaller the content of the treated magnet powders, it will be that much easier to provide the product with flame retardancy and because the treated magnet powders used according to this invention are originally high priced, a minimal amount of treated magnet powders should desirably be used, so long as the ultimately required magnetic characteristic can be met therewith. To effectively reduce the amount of the treated magnet powders used, providing the product in the form of an anisotropic magnet is effective. For example, for such uses as magnets for convergence correction in television sets, the amount of the treated magnetic powders may be reduced to 30% by volume or less. In that way, not only the flame retardancy may be imparted as intended by this invention, but excellent mechanical strength and favorable moldability may be provided as well.

In the bond magnet of this invention, a flame retarder is used. If any flame retarder is not used, even if the treated magnet powders used are improved in oxidation resistance, they are normally liable to combustion, providing only inadequate flame retardancy. The reason is that generally, bond magnets have large specific gravities and also high thermal conductivities and, moreover, contain large amounts of magnet powders and treated magnet powders which have small specific heats; therefore, unburnt parts tend to be heated to above the softening and decomposing temperature of the organic binder by the combustion heat at the time of initial ignition and combustion; then, the bond magnet drips, causing surrounding combustibles to catch fire, or the glowing after extinguishment to continue. Accordingly, it is necessary to put out the fire, being the heat source, as soon as the lighting is made, and so use of flame retarder is mandatory. As the flame retarder used according to this invention, a halogen containing flame retarder may be used in combination with a flame retarder aid and antiglowing agent, as required. A preferred flame retarder may be formulated by combination of aromatic bromine compound or chlorinated polycyclic or alicyclic compound and antimony trioxide. If the molding temperature of bond magnet is low, so that the halogen containing flame retarder will not decompose, of course, chlorinated or brominated aliphatic hydrocarbon compounds may be used. As such preferred halogen containing flame retarders, decabromodiphenyl ether, polybromostyrene tetrabromobisphenol A, tetrabromobisphenol S, "DECHLORANE 604", "DECHLORANE PLUS" ("DECHLORANE" is a Hooker Chemical's trade name), etc., may be illustrated. As the flame retarder aids, antimony trioxide, antimony pentoxide, etc., may be illustrated. And as the anti-glowing agents, zinc borate, phosphoric acid esters, etc., may be illustrated. The amount of the flame retarder used can not be unconditionally determined, greatly varying with types and proportions of other components of the bond magnet. The lower limit for its using amount should be arbitrarily set with the amenability of the organic binder to the process of making it flame retardant as the major index. The upper using amount limit may be set in terms of the moldability and mechanical strength of the bond magnet, because from further increase in its amount, further effect of flame retardancy improvement is not much expectable. Normally, proper amount of the flame retarder used according to this invention may fall in the range of 20 - 200 parts by weight of the amount of the organic binder as 100 parts by weight, 40 - 170 parts by weight being more preferable. Preferable ratio of the amount of the flame retarder used to that of the flame retarder aid is from 3 : 2 to 4 : 1. The anti-glowing agent should normally be used at a proportion of 0 - 50 parts by weight of the amount of the aforementioned flame retarder, depending on the amount of the treated magnet powders used, this effect being prominent, when more than 5 parts by weight of it is used.

In the bond magnets of this invention, with the aim at achieving improvement in the modability characteristic, mechanical porperties or thermal stability, plasticizer, lubricant, surface modifier for treated magnet powders, filler, stabilizer and other modifying additives may be jointly used, so long as they do not interfere with their flame retardancy.

For the molding of the bond magnets of this invention, proper method is selected from among various molding methods universally employed for molding bond magnets, taking account of the type of organic binder, content of treated magnet powders or the end to serve. They include, for example, injection, extrusion, compression and rolling. When bond magnets having magnetic anisotropy are desired to have, their molding is made, while applying a magnetic field which is higher than the inherent coercive force of the magnet powders used.

The bond magnets of this invention obtained in this way have both the excellent magnetic characteristic and flame retardancy which the rare earth/transition metal alloy magnets have. They are valuable as magnet parts for use in the perimeter of live parts in electric and electronic equipment.

In the following, modes of this invention will become more evident from the description taken in connection with its preferred embodiments, but this invention will not be bound thereby in any way.

### Reference example 1 (Preparation of treated magnet powders)

One hundred grams of SmCo₅ powders with their mean grain size 7µm, as measured by the air transmission method and 20mℓ of water having 0.4g sodium silicate dissolved therein were mixed and this mixture was stirred for 30 min in an inert gas atmosphere. Then sodium silicate was hardened on the magnet powders surfaces by adding to the mixture a dilute aqueous solution of phosphoric acid with stirring. The treated magnet powders, after filtered off, was cleaned with alcohol and, then, dried in a vacuum dryer at 60°C for 24 hr, yielding treated magnet powders A.

Besides, treated magnet powders B and treated magnet powders C were obtained similarly as above-descirbed, except that the amounts of sodium silicate used were set at 2.2g and 8.5g respectively.

If the magnet powders are regarded as spherical grains with grain diameter 7µm, the coating thickness of sodium silicate film of the treated magnet powders A may be determined as 0.22µm on the average.

### Reference example 2

One hundred grams of the same magnet powders as used in Reference example l was added to a tank holding 10 ℓ of an electroless nickel plating solution containing 10g of nickel sulfate which was held at 60°C in a warm bath. Plating was conducted while stirring the plating bath, the reaction being run until the plating solution was decolored into colorless and transparent. After accomplishing the reaction, the treated magnet powders and residual plating solution were separated by filtration, the treated magnetic powders thus obtained were water rinsed and, then, subjected to alcohol cleaning; thereafter, they were dried in a vacuum dryer at 60°C for 24 hr, yielding treated magnet powders D.

As the treated magnet powders A - D obtained in Refernece examples 1 and 2 were analyzed by a scanning electron microscope - X-ray microanalyzer, it was confirmed that sodium silicate and nickel respectively coated the magnet powder surfaces.

### Example 1 - 7

The treated magnet powders each of A - D obtained in Reference examples 1 and 2 and the organic binder, flame retarder and additives in the component ratio shown in Table 1 were respectively mixed with stirring and the mixture was melted by heating and kneaded for 10 min in a kneader type mixer. A lumpy kneaded product was taken out of the kneader and pulverized; thereafter, the powders obtained were molded in a heating press into a 0.8mm thick plate shape molding. From this plate shape molding, a test piece with 12.7mm width and 127mm length was prepared and with it vertical combustion test was conducted in accordance with the UL (Underwriters' Laboratories) Standard. The results given under the bottom column of Table 1 were obtained.

### Comparative example 1

A test piece was prepared exactly just as in Example 1, except that the same magnet powders provided for preparation of the treated magnet powders in Reference example 1 were used as they were, and it was put to a combustion test. The sample dripped at the first flame approach of the combustion test and, subsequently, it burned, while dripping, causing ignition of cotton placed downward thereof.

The residue remaining near the clamp and the dripped matters continued glowing for longer than 60 sec even after extinguishment of fire, with the glowing range tending to expand.

This Comparative example obviously shows that a large amount of flame retarder mixed will not provide adequate flame retardancy level.

### Comparative example 2

A test piece was prepared exactly just as in Example 1, except that no flame retarder was used, and it was put to a combustion test. This test piece violently dripped already at the first flame approach; the dripping on the burner put out the burner flame, thus making it impossible to conduct the combustion test. The dripped matter quickly taken off above the burner continued glowing for more than 60 sec.

As described in the foregoing, the bond magnets of this invention obtained from a composition prepared using specified treated magnet powders and a flame retarder give excellent flame retardancy and attain levels of V-2 or higher in the vertical combustion test according to the UL Standard. The flame retardant bond magnets of this invention are finding wide ranges of uses in the fields of electric and electronic equipment, etc., where flame retardancy is required.

## Claims

1. A flame retardant bond magnet comprising a flame retarder and an organic binder, besides alloy magnet powders with mean grain size 10µm or less represented by a general formula RM₅ (where R denotes a rare earth metal element, and M a transition metal element), which are coated on their surface with an oxidation resistant inorganic substance.

2. The magnet of Claim 1,wherein the rare earth metal element is samarium, and the transition metal element is cobalt.

3. The magnet of Claim 1,wherein the oxidation resistant inorganic substance is at least one member selected from among chromium, nickel, copper, zinc, silver, tin, gold, nickel - chrome alloy, nickel - copper alloy, silicate, borate, phosphate or borosilicate.

4. The magnet of Claim 1,wherein the silicate is at least one member selected from lithium, sodium, potassium or ammonium silicate.

5. The magnet of Claim 1,wherein when the oxidation resistant material is a metal or an alloy, it is coated on the alloy magnet powders by the metal film forming technique.

6. The magnet of Claim 1,wherein when the oxidation resistant material is an inorganic salt, a fine grained coating of said inorganic salt is formed on the surfaces of the alloy magnet powders while dispersing them into an aqueous medium in which the inorganic salt has been dissolved beforehand, and adding a hardener.

7. The magnet of Claim 6,wherein the hardener is at least one member selected from among silicofuluoride; mineral acid; oxide or salt of one of polyvalent metals comprising zinc, magnesium, zirconium, potassium and aluminum; and organic solvent.

8. The magnet of Claim 1,wherein the coating layer occupies at least 0.5% by volume of the coated alloy magnet powders.

9. The magnet of Claim 8,wherein the coating layer occupies 1 - 40% by volume of the coated alloy magnet powders.

10. The magnet of Claim 1,wherein the organic binder is at least one member selected from among polyvinyl chloride, vinyl chloride/vinyl acetate copolymer, polystyrene, acrylonitrile/styrene copolymer, 6-polyamide, 11-polyamide, 12-polyamide, polyethylene terephthalate, polybutylene terephthalate, polyphenylene oxide, polystyrene denatured polyphenylene oxide, polycarbonate, polysulfone, polyphenylene sulfide, polyallylate, thermoplastic polyimide, chlorinated polyethylene,chloroprene rubber, phenol resin, unsaturated polyester resin and epoxy resin.

11. The magnet of Claim 1, wherein the organic binder is mixed at 85 - 15% by volume in the total amount of said binder and the flame retarder, in proportion to 15 - 85% by volume of alloy magnet powders.

12. The magnet of Claim 1,wherein the flame retarder consists of a halogen containing flame retarder and a flame retarder aid.

13. The magnet of Claim 12,wherein the halogen containing flame retarder is at least one member selected from among decabromodiphenyl ether, polybromostyrene tetrabromobisphenol A, tetrabromobisphenol S, "DECHLORANE 604", "DECHLORANE PLUS" ("DECHLORANE" is a Hooker Chemical's trade name).

14. The magnet of Claim 12,wherein the flame retarder aid is at least one member selected from among antimony trioxide and antimony pentoxide.

15. The magnet of Claim 12,wherein the flame retarder further includes an anti glowing agent.

16. The magnet of Claim 15,wherein the anti- glowing agent is at least one member selected from among zinc borate and phosphoric acid ester.

17. The magnet of Claim 12,wherein the amount of the flame retarder is 20 - 200 parts by weight in proportion to 100 parts by weight of organic binder.

18. The magnet of Claim 12 wherein the halogen containing flame retarder and the flame retarder aid are contained in the ratio of 3 : 2 - 4 : 1.

19. The magnet of Claim 15,wherein the amount of the antiglowing agent is 0 - 50 parts by weight of the amount of the flame retarder.
